

Patented Nov. 11, 1924.

1,515,042

# UNITED STATES PATENT OFFICE.

AUGUST HECK, OF PHILADELPHIA, PENNSYLVANIA.

ELECTROLYTE AND COMPOSITION FOR FORMING THE SAME.

No Drawing.

Application filed August 22, 1923. Serial No. 658,670.

To all whom it may concern:

Be it known that I, AUGUST HECK, a citizen of the United States, residing at Philadelphia, in the county of Philadelphia and 5 State of Pennsylvania, have invented certain new and useful Improvements in Electrolytes and Compositions for Forming the Same, of which the following is a specification.

10 My invention relates to electrolytes, and compositions for forming the same, used in the electro-deposition of metals such as copper, zinc, brass, silver and gold.

Heretofore, in the art of electro-plating, 15 one of the most common forms of electrolytes or plating solutions consisted of a solution of cyanide of the metal to be deposited and cyanide of sodium or potassium, to which were sometimes added carbonate of soda, ammonium chloride, or other so-called 20 "conducting salts," the essential ingredients of the electrolyte being the cyanides, and the other materials being added in various quantities for the purpose of improving the 25 conductivity of the electrolyte according to various formulæ employed.

It frequently occurs, however, that, in the use of the cyanide solutions, either with or 30 without the addition of the conducting salts, the electrolyte will break down or decompose, resulting in the formation and deposition of scum or slime, and in some instances resulting in the precipitation of the 35 useful materials, which renders the electrolyte solution unfit for use.

The object of my present invention is to provide an improved form of electrolyte, and a prepared composition for use by the electro-plater in making the same, which 40 electrolyte will be more stable and durable than the various cyanide solutions at present in common use, and will better maintain its efficiency in use.

The nature and characteristic features 45 of my invention will be more readily understood from the following description of the improved form of electrolyte and the preferred form of the composition for preparing the same:

50 The general practice of preparing cyanide electrolytes consists in first dissolving a suitable quantity of cyanide of sodium or potassium in water, after which there is added to the solution the cyanide of the particular 55 metal to be deposited. For example, for

copper plating, copper cyanide is used; for zinc plating, zinc cyanide is used; for brass plating, a mixture of copper and zinc cyanides in the proper proportions is used; for silver plating, silver cyanide is used; 60 and for gold plating, gold cyanide is used. After the solution is prepared, there are sometimes added suitable quantities of "conducting salts," such as carbonate of soda, sal ammoniac, bisulphite of soda, etc., for the 65 purpose of increasing the conductivity of the solution.

Numerous formulæ have been evolved for the preparation of cyanide solutions, but it 70 is found in the practical use of the same that frequently, after the solution has been permitted to stand for a short time, the same will break down and decompose, the metals often being precipitated, scum will form 75 upon the surfaces of the anodes, and, when the plating is begun, instead of the metal being properly deposited, the solution will be found to be unfitted for the plating operation, requiring the same to be discarded 80 and a new solution made up, with the consequent expense and loss of time.

I have found that, in the use of cyanide 85 solutions, by the addition of a suitable quantity of boracic acid, the breaking down of the electrolyte will be largely eliminated, the same rendered more stable, the metal will be deposited more uniformly and in a heavier deposit in a given time, and the use of the so-called "conducting salts" may be 90 dispensed with.

For the purpose of making up the electrolyte, it will be found advisable to mix the boracic acid with the particular cyanide of the metal in a dry form, and furnish the 95 same to the electro-plater so mixed together. In making up this composition, there is preferably used about 50 parts of the boracic acid to each 100 parts of the metal cyanide.

When the electro-plater desires to make 100 up the bath, a suitable quantity of the prepared composition is used, which is mixed with the water in which the cyanide of sodium, or potassium, has previously been dissolved. While various strengths of the 105 solution may be used, according to the conditions under which the electro-plater is accustomed to work, the following formulæ will be found in practice to give satisfactory results:

For copper: Water, 1 gallon; sodium 110

cyanide, 6 ounces; prepared copper composition (copper cyanide and boracic acid) 12 ounces.

5 For zinc: Water, 1 gallon; sodium cyanide, 8 ounces; prepared zinc composition (zinc cyanide and boracic acid) 12 ounces.

10 For brass: Water, 1 gallon; sodium cyanide, 8 ounces; prepared copper composition (copper cyanide and boracic acid) 8 ounces; prepared zinc composition (zinc cyanide and boracic acid) 6 ounces.

15 For silver: Water, 1 gallon; sodium cyanide, 6 ounces; prepared silver composition (silver cyanide and boracic acid) 8 ounces.

20 For gold: Water, 1 gallon; sodium cyanide, 3 ounces; prepared gold composition (gold cyanide and boracic acid) 2 ounces.

25 By the employment of the prepared compositions for making up the electrolytes according to the above or any other desired formulae, the solutions may subsequently be brought to proper balance whenever it may be found necessary to replenish any of the materials which may have been used up. For example, if it should be found that, after use for a certain period, the electrolyte contains an excess of free cyanide of sodium, the same can be brought to proper balance by the addition of a suitable quantity of the prepared composition; or, if the electrolyte be found too rich in metal, it can be brought to a balance by the addition of a suitable quantity of cyanide of sodium, or potassium, as the case may be.

30 35 It will be found that, by the use of the electrolytes prepared as hereinbefore described, the stability and lasting qualities of the same will be greatly enhanced, the metal will be more uniformly and firmly deposited, and the electro-plating will be greatly improved generally.

40 When it will be found that in the use of electrolytes prepared as hereinbefore set forth, the addition of "conducting salts," such as carbonate of soda, sal ammoniac, etc., will not ordinarily be necessary, it should be understood that the same may be added if desired, without departing from the spirit and scope of my invention.

45 50 I am aware that boracic acid has heretofore been used in the formation of acid baths for use in nickel plating, but so far

as I am aware, the same has not heretofore been employed in the preparation of alkaline electrolytes in which cyanides of the metals to be deposited and cyanides of sodium, or potassium, are the principal active ingredients.

Having thus described the nature and characteristic features of my present invention, what I claim as new and desire to secure by Letters Patent is:

1. An electrolyte for use in electro-deposition of metals consisting of a solution in water of an appreciable amount of cyanide of an alkali metal, together with a mixture of solutions of cyanide of the metal to be deposited, and boracic acid, the latter ingredients being present in relatively large amounts.

2. An electrolyte for use in electro-deposition of metals consisting of a solution in water of an appreciable quantity of cyanide of an alkali metal and approximately double the quantity of a mixture of cyanide of the metal to be deposited and boracic acid, in the approximate proportions of one part of boracic acid to two parts of the cyanide of the metal.

3. A prepared composition for use in preparing cyanide solutions for electro-plating purposes, consisting of cyanide of the metal to be deposited, and a relatively large proportion of boracic acid.

4. A composition for use in preparing cyanide solutions for electro-plating purposes, consisting of cyanide of the metal to be deposited, and boracic acid, the boracic acid being approximately one-half the quantity of the cyanide of the metal.

5. The improvement in the art of electro-plating which consists in the employment in an electrolyte of the cyanide type of a quantity of boracic acid in a relatively large proportion.

6. The improvement in the art of electro-plating which consists in the employment in an electrolyte of the cyanide type of boracic acid in approximately one-half the amount of the cyanide of the metal.

In testimony whereof, I have hereunto signed my name.

AUGUST HECK.